



US007121323B2

(12) **United States Patent**  
**Weyer et al.**

(10) **Patent No.:** **US 7,121,323 B2**  
(45) **Date of Patent:** **Oct. 17, 2006**

(54) **METHOD AND DEVICE FOR THE  
CONTINUOUS CASTING AND DIRECT  
SHAPING OF A METAL STRAND, IN  
PARTICULAR A STEEL CAST STRAND**

(75) Inventors: **Axel Weyer**, Wuppertal (DE); **Dirk Letzel**, Ratingen (DE); **Horst Gärtner**, Düsseldorf (DE); **Wilfried Milewski**, Korschenbroich (DE); **Adolf Gustav Zajber**, Langenfeld (DE)

(73) Assignee: **SMS Demag AG**, Düsseldorf (DE)

(\*) Notice: Subject to any disclaimer, the term of this patent is extended or adjusted under 35 U.S.C. 154(b) by 64 days.

(21) Appl. No.: **10/498,650**

(22) PCT Filed: **Jan. 30, 2003**

(86) PCT No.: **PCT/EP03/00915**

§ 371 (c)(1),  
(2), (4) Date: **Jun. 10, 2004**

(87) PCT Pub. No.: **WO03/070399**

PCT Pub. Date: **Aug. 28, 2003**

(65) **Prior Publication Data**

US 2005/0011629 A1 Jan. 20, 2005

(30) **Foreign Application Priority Data**

Feb. 22, 2002 (DE) ..... 102 07 597  
Aug. 8, 2002 (DE) ..... 102 36 368

(51) **Int. Cl.**

**B22D 11/12** (2006.01)

(52) **U.S. Cl.** ..... **164/476; 164/477**

(58) **Field of Classification Search** ..... **164/455,  
164/476, 477, 417**

See application file for complete search history.

(56)

**References Cited**

**U.S. PATENT DOCUMENTS**

3,589,429 A 6/1971 Schoffmann

**FOREIGN PATENT DOCUMENTS**

|    |         |         |
|----|---------|---------|
| DE | 1817277 | 11/1970 |
| DE | 2042546 | 3/1972  |
| DE | 4436328 | 4/1995  |
| EP | 0545104 | 6/1993  |

(Continued)

**OTHER PUBLICATIONS**

Patent Abstracts of Japan, vol. 007, No. 269 (M-269), Nov. 30, 1983  
& JP 58 148059 A (Nippon Kokan KK), Sep. 3, 1983.

(Continued)

*Primary Examiner*—Len Tran

(74) *Attorney, Agent, or Firm*—Friedrich Kueffner

(57)

**ABSTRACT**

The invention relates to a method and a continuous casting device for the direct shaping of a metal strand, in particular a steel cast strand (1) of any format (1d). According to said method, the cast strand (1) is only cooled by a liquid coolant (4) in longitudinal sections (6), where the interior of the cast strand (1) remains liquefied and the temperature of the cast strand (1) in a transition zone (7) upstream of, in and/or downstream of a bending and straightening unit (8) is evened out by an insulation of the exterior surface (1b), essentially without the use of a liquid coolant (4), and by progressive thermal radiation. The cast strand (1) is shaped in a dynamically variable reduction section (9) as a result of the compressive strength that is measured on individual shaping rolls (10) or roll segments (11), depending on the compressive force that can be locally applied.

**13 Claims, 8 Drawing Sheets**



**US 7,121,323 B2**

Page 2

---

FOREIGN PATENT DOCUMENTS

|    |         |         |
|----|---------|---------|
| EP | 0804981 | 11/1997 |
| EP | 0903192 | 3/1999  |
| EP | 0980295 | 2/2000  |
| WO | 0234432 | 5/2002  |

WO

0298587 12/2002

OTHER PUBLICATIONS

Patent Abstracts of Japan, vol. 011, No. 348 (M-642), Nov. 14, 1987  
& JP 62 130759 A (Sumitomo Metal Ind. Ltd), Jun. 13, 1987.

FIG. 1



FIG. 2



FIG. 3



FIG.4



FIG.5





FIG.10



FIG.11



FIG. 12B

A - A



FIG. 12A

A - A



FIG. 13C



with insulation

FIG. 13B



drive position

FIG. 13A



normal position

**METHOD AND DEVICE FOR THE  
CONTINUOUS CASTING AND DIRECT  
SHAPING OF A METAL STRAND, IN  
PARTICULAR A STEEL CAST STRAND**

The invention concerns a method and a device for the continuous casting and direct deformation of a metal strand, especially a cast steel strand, which has a rectangular format or the format of a bloom, preliminary section, billet, or round, is guided in a curved strand guide after the continuous casting mold, subjected to secondary cooling with a liquid coolant, and prepared in an automatically controlled way for the deformation pass at a uniform temperature field in the strand cross section.

In general, in the continuous casting of different steel grades and dimensions or formats, one's attention is directed at the strand shell growth during secondary cooling and at the position of the tip of the liquid crater in a deformation line. It is known, for example, from EP 0 804 981 that the cast strand can be sufficiently compressed in the deformation line to produce the desired final thickness. However, this makes it necessary to determine the position of the tip of the liquid crater, based upon which the deformation force is applied horizontally along a wedge-shaped surface. However, a process of this type is relatively coarse and does not take into account the state of the microstructure that is to be expected. The reason lies in the unsatisfactory heat distribution due to unfavorable cooling and uniform strand support with nonuniform heat dissipation from the strand cross section. Adjustment of the secondary cooling to the strand support does not occur, either. To improve these conditions, it was proposed in German Patent Application 100 51 959.8, which has not been pre-published, that the secondary cooling be analogously adapted in its geometric configuration to the solidification profile of the cast strand on the following traveling length of the cast strand. The strand support is likewise analogously reduced as a function of the solidification profile of the cast strand at the respective travel length. In this connection, with increasing travel length, the corner regions of the cast strand cross section are less cooled than the middle regions. In the realization of this process, the spray angles of the spray jets in the secondary cooling are adjusted to the strand shell thickness in such a way that a low spray angle is assigned to a decreasing liquid crater width. A significant equalization of the temperature in the strand cross section over layers of the strand cross section is already achieved by these measures.

With this knowledge, the inventor of the above-cited, unpre-published patent application further recognized that the manner in which the process of so-called soft reduction of the cast strand is carried out must be further optimized. This recognition is based on the fact that high deformation resistance due to unfavorable temperature distribution in the cast billet or in the cast preliminary section with variable ductility causes variable deformation resistance and variable strain and thus leads to cracking.

An improvement of the internal quality of cast strands with different cross-sectional shapes and dimensions, especially with respect to positive segregation, core porosity, and core breakdown, requires a reduction process in the solidification range. The previously used procedure, e.g., with billet cross sections, leads to circular solidification with circular isotherms in the cross section, which develop in the region of the bending and straightening driver. Since only a reduction in the core is possible with this type of temperature distribution, only a mechanically influenced final solidification is achieved. However, the results are unsatisfactory and

subject to very strong fluctuations. The reason is that the region of final solidification is very difficult to determine.

The objective of the invention is to produce the necessary temperature distribution in the cast strand and thus to optimize the deformation pass and to obtain a useful microstructure of the final solidification at the end of the deformation pass.

In accordance with the invention, this objective is achieved by cooling the cast strand with a liquid coolant only in the longitudinal sections in which the cast strand is predominantly liquid in the cross section, by equalizing the temperature of the cast strand in a transition zone before, in, and/or after a bending-straightening unit by insulation of the exterior surface that is radiating heat, basically without the use of a liquid coolant, and further equalizing the temperature by heat radiation in zones, and by deforming the cast strand on a dynamically variable reduction line on the basis of the compressive strength measured by individual deforming rolls or roll segments, depending on the compressive force that can be locally applied. The advantages are a casting and cooling process that better prepares the deformation process with a varied solidification or temperature profile in the strand cross section and a reduction process with a continuous or variable course of reduction, which lead to a largely defect-free microstructure of the final solidification.

The deformation process can be further optimized if the temperature field consists of elliptical, horizontally oriented isotherms.

In addition, an advantageous refined condition is created if the temperature pattern is uniformly formed in the transverse and longitudinal direction of the core region in the strand cross section.

A procedure of this type is further assisted by compressing the cast strand on the dynamically variable reduction line in the core region in the transverse and longitudinal direction.

The edge lengths of a polygonal strand cross section play an important role in the cooling of the cast strand. Therefore, it is quite important for the deformation to be carried out as a function of the strand format, the strand dimensions, and/or the casting speed.

Basically, the deformation on the deformation line can be carried out by two systems, namely, deformation by point pressing by individual deforming rolls or by approximate surface pressing by roll segments.

Another embodiment of the method in the case of surface pressing consists, in the case of deformation by roll segments, in the use of different conicities for different steel grades in the adjustment of the roll segments.

Another very important aspect of the invention is the automatic control and regulation, i.e., the measuring and automatic control engineering of the deformation operation. To this end, the method described above provides automatic control by adjusting several roll segments in the normal position or with constant conicity or with progressive conicity or with variable conicity, which can be adjusted by the automatic control system. The deformation can then be carried out accordingly, depending on the deformation resistance that is determined.

In addition, the continuous or variable course of reduction is assisted by automatically controlling the compression of the core region of the cast strand by determining its deformation resistance and/or the distance traveled by the strand.

A less mechanically influenced final solidification is then achieved by compressing approximately horizontal layers in the strand cross section, which have the same isotherms, during the deformation.

A shape-preserving supportive measure that can be used here consists in supporting and guiding the cast strand, at least during the deformation, by support rolls that lie against the two lateral faces.

In this regard, the total deformation energy supplied can be distributed by adjusting the rate of the reduction process to 0–14 mm/m.

The process of the general type described above for continuous casting and direct deformation is designed in such a way with respect to the automatic control engineering that the instantaneous deformation rate is adjusted to the given temperature of the cast strand and/or to the casting rate by continuously measuring the deformation resistance on the individual deforming rolls or on the individual roll segments, determining the position of the tip of the liquid crater on the basis of the given contact force, and automatically controlling the volume of coolant, the contact force, the casting rate, and/or the run-out rate of the deformed cast strand.

Fixed initial values can be additionally obtained by initially assigning a deformation rate to each deforming roll or each roll segment in a fixed relationship.

The device of the general type described above for continuous casting with direct deformation is designed in such a way that the curved strand guide with the spray device for liquid coolant is followed by a predominantly dry zone, which operates for the most part without liquid coolant and serves as insulation against the elimination of radiant heat and systematically surrounds the cast strand, and that a reduction line is provided, which consists of individual, hydraulically adjustable deforming rolls or several hydraulically adjustable roll segments and precedes, coincides with, or follows the region of the bending-straightening unit.

In the event of a shift of the tip of the solidification cone, a correction can be made by displacing roll segments that are arranged in the direction of strand travel next to one or more stationary bending-straightening units either in the direction of strand travel or in the opposite direction.

Different deformation forces can be applied within the roll segments if each reduction roll segment has at least two pairs of rolls, of which at least one adjustable deforming roll is equipped with a piston-cylinder unit.

In the case of a rigidly installed lower pair of deforming rolls or a rigid lower roll segment, the different deforming forces can also be produced by equipping the upper, adjustable deforming roll or the upper, adjustable roll segment each with two piston-cylinder units per pair of rolls, such that the piston-cylinder units are arranged in succession on the centerline or are arranged in pairs outside the centerline.

In another measure for an advantageous deformation line, the roll spacing in a roll segment is selected as a close spacing in the range of 150–450 mm.

It is further proposed that bending-straightening units installed in the region of the radiation insulation are likewise insulated from heat radiation by the cast strand.

Embodiments of the method and device of the invention with the deformation line are illustrated in the drawings and explained in greater detail below.

FIG. 1 shows a side view of a continuous casting device, e.g., for billet formats.

FIG. 2 shows an effective strain lying in the plane with an elliptical temperature field in stationary operation.

FIG. 3 shows a perspective view of a cutaway portion of effective strain with an elliptical temperature field after the first pass in the deformation line.

FIG. 4 shows a first system of soft reduction with individual deforming rolls.

FIG. 5 shows a second system of the deformation line with roll segments.

FIGS. 6 to 9 show different conicity settings of the roll segments.

FIG. 10 shows a side view with several bending-straightening units and with the deformation line.

FIG. 11 shows an alternative embodiment of the deformation line with individual driven deforming rolls.

FIG. 12A shows a side view of another alternative embodiment of the bending-straightening units and the roll segments.

FIG. 13A shows a deformation stand in normal position.

FIG. 13B shows a deformation stand in drive position.

FIG. 13C shows the deformation stand with insulation.

FIG. 1 shows a continuous casting device for the example of a billet strand format 1d of a cast strand 1. However, the strand cross section 1a could also have a rectangular format or the format of a bloom, preliminary section, or round.

The molten steel material from a continuous casting mold 2 is subjected to secondary cooling with liquid coolant 4, e.g., water, in a (curved) strand guide 3 and adjusted to a uniform temperature field 5 in the strand cross section 1a by an automatic control system (cf. FIG. 2 also). This results in a liquid-cooled longitudinal section 6 with a solid shell and a liquid core region 1c.

The curved strand guide 3 with a spray device 4a for the liquid coolant 4 is followed by a predominantly dry zone 24, which operates for the most part without liquid coolant 4 and serves as insulation 25 against the elimination of radiant heat and systematically surrounds the cast strand 1, such that the possible length of insulation in the longitudinal region indicated by arrows is maintained as a function of the strand format 1d, the dimensions, the casting speed, and other parameters of this kind. The dry zone 24 can, for example, as shown in the drawing, extend over the liquid/dry transition zone 7 as far as the bending-straightening unit 8 with a preceding or following reduction line 9. The reduction line 9 consists of individual, hydraulically adjustable deforming rolls 10 or of several hydraulically adjustable roll segments 11, as shown in FIG. 11.

The method based on the continuous casting machine for molten steel explained above is now carried out in such a way (FIGS. 2 and 3) that the cast strand 1 is used by the liquid coolant 4 only in liquid-cooled longitudinal sections 6 in which the cast strand is still liquid or predominantly liquid in the cross section 1a. In a transition zone 7 before, in, and/or after the bending-straightening unit 8, the heat-radiating exterior surface 1b is thermally insulated basically without the use of the liquid coolant, so that heat radiation in such zones results in less cooling and/or support of colder cross-sectional parts, e.g., the corner edges 1f, than of other cross-sectional parts that are connected with the still hot or liquid core region 1c. This equalizes the heat distribution in the strand cross section 1c. The temperature field 5 is obtained with elliptical, essentially horizontally oriented isotherms 12 (FIGS. 2 and 3).

The cast strand 1 is deformed on the basis of this improved temperature distribution on a dynamically variable reduction line 9 and on the basis of the compressive strength measured by the individual deforming rolls 10 or one or more roll segments 11, depending on the compressive force that can be applied locally.

The temperature field 5 (FIG. 2) is formed uniformly in the transverse and longitudinal direction 1e of, the core region 1c in the strand cross section 1a.

On the basis of the isotherms 12, the cast strand 1 can be compressed on the dynamically variable reduction line 9 in the core region 1c in the transverse and longitudinal direc-

tion 1e (FIGS. 4 and 5). The deformation is carried out as a function of the strand format 1d, the strand dimensions 14, and/or the given casting speed in the longitudinal direction 13. The deformation can also be carried out by line pressing (FIG. 4) by individual deforming rolls 10, or by approximate surface pressing by several roll segments 11 (FIG. 5). In this connection, the core region 1c is compressed to a liquid crater tip 1g in each case. In the case of deformation by roll segments 11, different conicities 15 can be used for different grades of steel by suitable adjustment of the roll segments 11.

Examples of different conicities 15 are shown in FIGS. 6 to 9. FIG. 6 shows the "normal position" 16 of the roll segments 11, i.e., the conicity is 0°. Nevertheless, compression occurs. In FIG. 7, a constant conicity 17 is set for all roll segments 11. On the other hand, FIG. 8 shows a changing angle of conicity from one roll segment 11 to the next in the sense of progressive conicity 18. It is also possible, as shown in FIG. 9, to set a variable conicity, depending on the position of the tip of the liquid crater 1g.

The compression of the core region 1c (FIGS. 4 and 5) of the cast strand 1 by the pressure cones 1h is initially controlled by determining the given deformation resistance and/or a strand distance 20 that has been traveled (distance determination). The formation of the temperature field 5 uniformly in the transverse and longitudinal direction 1e of the core region 1c is especially effective here. So-called optimized isotherms 12 are obtained in this way. The isotherms 12 run especially flat in this case. The deformation resistance can be measured, for example, under an individual deforming roll 10 by measurement of the hydraulic pressure in a hydraulic line or other hydraulic component.

Layers 21, which, advantageously, are approximately horizontal and have the same isotherms 12, are compressed in the transverse direction 1e of the strand cross section 1a (cf. FIGS. 2 and 3). During the compression of the core porosities, existing segregations can be eliminated at the same time. The given layer 21 that is still hotter and thus softer yields during this compression process.

As FIG. 12B shows, it is advantageous to install support rolls 22 that rest on the two exterior surfaces 1b during the deformation to prevent spreading of the cast strand 1 on its exterior surface 1b. The rate of the reduction process can be adjusted and automatically controlled to (instantaneously) 0–14 mm per running meter of cast strand 1.

Furthermore, the automatic control process for a soft reduction takes place: The instantaneous deformation rate is adjusted to the given temperature of the cast strand 1 and/or the (set) casting speed (e.g., 3.2 m/min). To this end, the deformation resistance is continuously measured (e.g., by the hydraulic pressure) on the individual deforming rolls 10 or on the individual roll segments 11. The position of the tip 1g of the liquid crater is determined on the basis of the given contact force that is determined, and, for example, the volume of the sprayed coolant 4, the contact force, the casting speed, and/or the run-out rate of the deformed cast strand 1 is automatically controlled, so that the tip 1g of the liquid crater reaches a desired position within the thus dynamic, variable reduction line 9. A deformation rate can be initially assigned to each individual deforming roll 10 or each roll segment 11 in a fixed relationship according to the conicity system of FIGS. 6 to 9.

The essential assemblies of the deformation line 10 are shown in FIGS. 10 to 13C.

In FIG. 10, several roll segments 11 are located next to one or more stationary bending-straightening units 8 on a common base plate 26. The base plate 26 with the bending-straightening units 8 and the (four) roll segments 11 shown in the drawing can be displaced back and forth to a limited

extent in the region of a varied position of the tip 1g of the liquid crater and accordingly is connected to the automatic control system.

Each of the (six) reduction roll segments 11 is equipped with at least two pairs of rolls 11a. At least one adjustable deforming roll 10 is equipped with a piston-cylinder unit 27.

As FIGS. 12A and 12B show, in the case of a rigid lower pair 11a of deforming rolls or a rigid lower roll segment 11, the upper, adjustable deforming roll 10 or the upper, adjustable roll segment 11 can each be provided with two piston-cylinder units 27 arranged in succession on the centerline 28 or arranged in pairs outside the centerline 28.

The roll spacing 29 (FIGS. 4 and 5) on a roll segment 11 is selected as a close spacing in the range of 200–450 mm at a roll diameter of 230 mm (roll segment 11) or 500 mm (individual deforming roll 10).

FIGS. 13A, 13B, and 13C show an individual roll segment 11 of this type for a billet format. In FIG. 13A, the drive 30 and the pair of rolls 11a are in the normal position. In FIG. 13B, the pair of rolls 11a and the drive are shown in the drive position. FIG. 13C shows the insulation 25 in the area of the reduction line 9.

The invention can also be used to advantage for the entire spectrum of steel grades, such as special steels, high-grade steels and stainless steels.

The invention claimed is:

1. Method for the continuous casting and direct deformation of a metal strand, especially a cast steel strand (1), which has a rectangular format or the format of a bloom, preliminary section, billet, or round, is guided in a curved strand guide (3) after the continuous casting mold (2), subjected to secondary cooling with a liquid coolant (4), and prepared in an automatically controlled way for the deformation pass at a uniform temperature field (5) in the strand cross section (1a), such that the cast strand (1) is cooled with a liquid coolant (4) only in the longitudinal sections (6) in which the cast strand (1) is liquid in the cross section (1a), wherein the temperature of the cast strand (1) is equalized in a transition zone (7) before, in, and/or after a bending-straightening unit (8) by insulation of the exterior surface (1b) that is radiating heat, without the use of a liquid coolant (4), and further equalized by heat radiation in zones in such a manner that colder corner regions (1f) are cooled and supported less than other cross-sectional parts, which are connected with the still hot core region (1c), until the temperature field (5) consists of elliptical, horizontally oriented isotherms (12), and that the cast strand (1) is deformed on a dynamically variable soft reduction line (9) on the basis of the compressive strength measured by individual deforming rolls (10) or roll segments (11), depending on the compressive force that can be locally applied.

2. Method in accordance with claim 1, wherein the temperature pattern (5) is uniformly formed in the transverse and longitudinal direction (1e) of the core region (1c) in the strand cross section (1a).

3. Method in accordance with claim 1, wherein the cast strand (1) is compressed on the dynamically variable reduction line (9) in the core region (1c) in the transverse and longitudinal direction (1e).

4. Method in accordance with claim 1, wherein the deformation is carried out as a function of the strand format (1d), the strand dimensions (14), and/or the casting speed.

5. Method in accordance with claim 1, wherein the deformation is carried out by pressing at points by individual deforming rolls (10) or by approximate surface pressing by roll segments (11).

6. Method in accordance with claim 5, wherein, in the case of deformation by roll segments (11), different conicities (15) are used for different steel grades in the adjustment of the roll segments (11).

7. Method in accordance with claim 1, wherein several roll segments (11) are adjusted in the normal position (16) or with constant conicity (17) or with progressive conicity (18) or with variable conicity (19).

8. Method in accordance with claim 1, wherein the compression of the core region (1c) of the cast strand (1) is automatically controlled by determining its deformation resistance and/or the distance (20) traveled by the strand.

9. Method in accordance with claim 1, wherein approximately horizontal layers (21) in the strand cross section (1a), which have the same isotherms (12), are compressed during the deformation.

10. Method in accordance with claim 1, wherein, at least during the deformation, the cast strand (1) is supported and guided by support rolls (22) that lie against the two exterior surfaces (1b).

11. Method in accordance with claim 1, wherein the rate of the reduction process is adjusted to 0–14 mm/m.

12. Method in accordance with claim 1, wherein the instantaneous deformation rate is matched to the given temperature of the cast strand (1) and/or to the casting rate by continuously measuring the deformation resistance on the individual deforming rolls (10) or on the individual roll segments (11), determining the position of the tip (1g) of the liquid crater on the basis of the given contact force, and automatically controlling the volume of coolant, the contact force, the casting rate, and/or the runout rate of the deformed cast strand (1).

13. Method in accordance with claim 12, wherein a deformation rate is initially assigned to each deforming roll (10) or each roll segment (11) in a fixed relationship.

\* \* \* \* \*